

April 20, 1937.

G. J. ESSELEN ET AL

2,078,214

U. S. PATENT OFFICE  
PROCESS OF MAKING COLORED SHEETS OF CELLULOSE  
ESTERS, SYNTHETIC RESINS, AND THE LIKE  
Filed June 17, 1935

Filed June 17, 1935



### *Inventors:*

Inventors:

Gustavus J. Esselen and  
Jacob Curie  
Dike, Calm & Gray  
Attorneys.

## UNITED STATES PATENT OFFICE

2,078,214

PROCESS OF MAKING COLORED SHEETS  
OF CELLULOSE ESTERS, SYNTHETIC  
RESINS, AND THE LIKE

Gustavus J. Esseen, Swampscott, and Jacob Lurie, Springfield, Mass., assignors to The Fiberloid Corporation, Indian Orchard, Mass., a corporation of Massachusetts

Application June 17, 1935, Serial No. 27,012

1 Claim. (Cl. 91—68)

The present invention relates to a novel process of making sheets or a web of cellulose esters, synthetic resins or like plastic materials in colors or having ornamental effects.

At the present time sheets of cellulose ester plastics or the like can be made by a continuous process which forms a web and seasons it, but it has not been practical to make a wide variety of colors and shades of stock in this way since the process is economical only for large batches which provide long runs and do not require frequent cleaning of the machines. Only small quantities of any particular color are ordinarily required, but many colors, and shades are necessary. Accordingly, colored sheet stock has heretofore been made entirely by the cake or block process, in accordance with which a cake or block is formed, is then sliced into sheets and the seasoning of the sheets completed. This process is exceedingly slow and expensive. Our novel process makes it possible to produce colored sheet stock by a continuous process and without resorting to the cake process and at much less expense.

In accordance with the novel process, we make by the continuous process a transparent, translucent or white opaque sheet or web from cellulose esters, synthetic resins or like plastic materials and thereafter apply simultaneously on both sides of the web a thin coating of a suitable colored or ornamental finishing liquid. When so treated the sheet has the appearance of a sheet made entirely from colored stock. In addition very beautiful effects may be obtained by choosing the colors to be applied to the face or faces of the base material. It will be understood that the base material may be of any desired appearance and the surface coating likewise of any desired appearance, and in general in this specification we have used the word color to include clear transparent, white opaque and even black and have not limited it to the spectrum colors.

The novel process greatly reduces the cost of colored sheet stock since the sheet forming machine may be run continuously to form the colorless, i. e. transparent, translucent or white opaque, base material and this material may subsequently be colored or coated or ornamented as desired.

The surface coatings applied may themselves be transparent translucent or opaque, they may be of a single color or a non-uniform mixture of colors, or they may contain ornamental material in suspension, as, for instance, pearl essence,

metallic scales, and the like and the opposite sides of the sheet may be given the same or different colors or ornamentation. Our invention, therefore, makes it possible to produce by the continuous process many, if not all, of the colored and pearl effects, either plain or mottled which are now produced by the cake process and thus to take advantage of the very great economies of the continuous process. Furthermore, certain effects can be produced by our process which are not now possible with the cake process.

The improved process consists in general in preparing a coating liquid from a mixture of a suitable carrier liquid, such as lacquer, and the desired coloring matter; flowing the colored coating liquid onto a bath of suitable liquid, for instance water, to form a film of desired thickness; then linearly passing the sheet to be coated continuously down through the film of coating liquid into the bath at a speed such that the film of coating material on each side of the sheet will be drawn against the sheet continuously; and carrying the sheet through the bath and out of it at a place where the bath is free from the coating film. In practice, it is desirable to employ a tank divided into two parts or cells by a partition which does not extend to the bottom of the tank. In this way the coating is applied simultaneously to both sides of the sheet but is not injured when it is removed from the tank.

In practicing our invention, we prefer to harden somewhat the film on the surface of the bath by removing some of the solvent contained in the coating material just before it contacts with the sheet of base material. When this is done, we treat the surface of the sheet with a small quantity of some suitable solvent or softening agent which activates the surface of the sheet and renders it more easily adherent to the film taken from the surface of the bath. By this treatment, which is not claimed herein as it is made the subject of a companion application, a tougher film is formed and the sheet may be passed through the bath at substantially greater speed.

Referring to the drawing, the figure is a vertical section of a machine illustrating somewhat diagrammatically our invention.

At 10 is shown a machine having a nozzle 11 for forming a continuous sheet or web 13. From the die, the web passes through suitable driers 14 in which the solvent is extracted and the stock is seasoned. The web thus formed is, for instance, of transparent cellulose ester plastic and 55

is to be converted into a blue opaque material. The web 13 is fed lineally by positively driven feed rollers 15 and 16 downward into the bath 17 contained in the tank 18. The tank 18 is provided with a partition 19 which divides it into two cells. The partition 19 extends downward below the level of the bath 17 in the tank, having due regard to variations in level which may take place. Above the entering cell, which is at the left of the partition, we place two troughs 20 and 21 which supply the coating material for the web. These troughs, or other suitable supply mechanism, are arranged to supply the coating material at a uniform regulatable rate. The coating material, which is preferably a suitable nitrocellulose lacquer containing the desired coloring material, floats on the surface of the bath and spreads out forming a film thereon. For making light blue opaque stock, this film may be made satisfactorily of a lacquer containing 10 ounces of titanium dioxide, 1 ounce of Chinese blue in each gallon of clear lacquer. The clear lacquer is made by dissolving 1 pound of  $\frac{1}{2}$  second nitrocellulose and  $\frac{1}{3}$  of a pound of dibutyl phthalate in 1 gallon of solvent mixture. A convenient solvent mixture is composed of 40 parts of toluol, 30 parts of ethyl acetate, 20 parts of butyl acetate and 10 parts of butanol, all the parts being by volume. The bath on which the coating liquid is floated is of some liquid which is not a solvent for the solid constituents of the coating liquid, although it may be miscible with one or more of the solvents used to make up the coating liquid. For ordinary purposes, water is satisfactory. At 22 and 23 are shown two air nozzles which blow warm air gently on the surface of the film and remove some of the solvent and harden and toughen the film slightly as already described. If preferred, the bath may be heated slightly. The web 13 passes lineally down through the film 24 on the surface of the bath and the film adheres to each side of the web. As the web or continuous sheet lineally progresses downward through

the bath, the film is drawn by its own toughness and cohesion toward the sheet so that both sides of the sheet are continuously and smoothly coated. At 25 and 26 are shown spray nozzles which apply a fine mist of a suitable solvent, for instance butyl acetate, to the sides of the sheet after it leaves the feed rolls 15 and 16 and before it comes in contact with the film of coating material on the surface of the bath. After passing through the film 24 of coating material on the surface of the bath the web passes under the partition 19 and then is led upward through the right hand cell of the bath emerging at 27. There is no film of coating material on this portion of the bath. After emerging from the bath, jets of warm air are directed by nozzles 28 and 29 against the opposite sides of the sheet, drying and hardening the film of coating material sufficiently so that it will not be marred by or adhere to the rollers 30 and 31 over which the material is led. By giving the rollers 15 and 16 and 30 and 31 the same peripheral speeds, a festoon is formed passing under the partition and the sheet is guided through the bath without coming in contact with any object from the time it leaves the feed rollers 15 and 16 until it is received by the delivery rollers 30 and 31.

What we claim is:

The improvement in the continuous process of making sheet stock from cellulose esters, synthetic resins and the like whereby a continuous web of said material is produced which comprises supplying to a bath a floating film of colored liquid capable of adhering to the web, feeding the web lineally through the film into the bath, thereby causing the floating film to adhere to both sides of the web, thereafter feeding the coated web out of the bath at the place where the bath is not covered with coating material and drying the coated web.

GUSTAVUS J. ESSELEN.  
JACOB LURIE.